

# United States Patent

[19]

Dodson et al.

[11] 3,850,828

[45] Nov. 26, 1974

[54] **GREASE COMPOSITION**

[75] Inventors: **Stanley Charles Dodson, Leatherhead; Robert Henry Newman, Weybridge, both of England**

[73] Assignee: **The British Petroleum Company Limited, London, England**

[22] Filed: **Nov. 27, 1972**

[21] Appl. No.: **309,680**

[30] **Foreign Application Priority Data**

Nov. 29, 1971 Great Britain ..... 55306/71

[52] **U.S. Cl.** ..... 252/59

[51] **Int. Cl.** ..... C10m 5/10, C10m 7/14

[58] **Field of Search** ..... 252/59, 56 S

[56] **References Cited**

UNITED STATES PATENTS

|           |         |                      |        |
|-----------|---------|----------------------|--------|
| 3,290,244 | 12/1966 | Polishuk et al. .... | 252/59 |
| 3,392,119 | 7/1968  | Mitacek ....         | 252/59 |

*Primary Examiner*—Daniel E. Wyman

*Assistant Examiner*—I. Vaughn

*Attorney, Agent, or Firm*—Morgan, Finnegan, Durham & Pine

[57] **ABSTRACT**

A grease composition consists of a lubricating base oil thickened e.g. to a penetration value of above 310, by a mixture of atactic polypropylene of Melt Viscosity Index above 50 and a polyethylene preferably a high density polyethylene.

**5 Claims, No Drawings**

## GREASE COMPOSITION

This invention relates to a polymer-thickened grease composition more particularly it relates to a polyolefin-thickened grease composition.

It is known to thicken lubricating oils into greases using particular polyethylenes, either alone or in admixture with other thickeners such as alkali metal soaps, e.g. as described in UK Patent No. 986192.

We have found that greases thickened by polyethylene tend to have a "grainy" structure which is very difficult to convert to a smooth grease, and more satisfactory greases can be formed by use of a mixture of olefin polymers.

According to the invention there is provided a grease composition comprising a mineral or synthetic lubricating oil or blends thereof thickened to a grease consistency by a mixture of a polyethylene and an atactic polypropylene of Melt Index above 20.

The polyethylene which is used is preferably a high density polymer e.g. of density above 0.94 gm/cc, and in order to produce a grease with a lower polymer content the higher molecular weight polymers are preferred. However the lower molecular weight polymers tend to form greases which have a smoother structure, or one which can be easily smoothed, so the choice of polymer will tend to depend on the use to which the grease is to be put. However for general purposes, such as greases for enclosed gear lubrication, a lower content of polymer is preferred. Suitable polyethylenes are sold under the Trade Mark "Rigidex".

The Melt Index of the polypropylene is preferably greater than 50. In the atactic polypropylene the amount of isotactic polypropylene is preferably below 10%. The Melt Index of the polypropylene can be ob-

ylene is preferably 1:1 to 10:1 more preferably 2:1 to 5:1.

The grease compositions of the present invention preferably have a penetration above 300, more preferably of 310-500.

The penetration of the greases can be measured by Test Method ASTM 217-68.

The invention will now be described with reference to the following Example.

## EXAMPLE

Greases were prepared from two different lubricating base oils by heating half the total quantity of oil and the polyethylene to 100°C. The atactic polypropylene was slowly added whilst heating to 150°C. mins.

The batch was held at 150°C for 1 hour, to allow the polymers to swell and partially dissolve. The batch was heated to 180°C and held at this temperature for at least 30 mins to give a complete solution of the polymers. The rest of the lubricating oil was added and the batch cooled as quickly as possible to form a grease. The grease was circulated through a homogeniser at 80°C to give a smooth grease.

Tables 1 and 2 give information on the materials used in the forming of greases in Table 3. Table 4 shows the effect of Melt Index on Grease Structure.

In the Tables, smooth means a grease having a smooth consistency and is substantially homogeneous, grainy means having the appearance of grains or particles in the grease, and rubbery means a more cohesive and spongy or elastic structure than the well known "buttery" structure of most lubricating greases. In addition removing some of such a grease from the bulk forms strings still attached to the bulk of the grease, the strings having elastic properties.

TABLE 1

| DATA ON POLYMERS      |      |            |         |            |              |                  |
|-----------------------|------|------------|---------|------------|--------------|------------------|
| Polymer               | Type | Trade Name | Grade   | Melt Index | Density g/ml | Molecular weight |
| Atactic Polypropylene | B    | —          | 0 - 20  | 0 - 20     | 0.87         | 9,000/10,000     |
|                       |      |            | 20 - 50 | 20 - 50    | 0.87         | (Isotactic)      |
|                       |      |            | >50     | >50        | 0.87         | content          |
|                       |      |            |         |            |              | about            |
|                       |      |            |         |            |              | 6% )             |
| Polyethylene          | II   | Rigidex    | XGR 369 | —          | 0.96         | 150,000          |
| III                   | do.  | Type 9     | —       | 0.9        | 0.96         | 88,000           |
| IV                    | do.  | Type 50    | 5       | 5          | 0.96         | 70,000           |

Melt Index: BS 2782, Method 1050 for polyethylene

ASTM D 1238 for polypropylene at 190°C

Molecular Weight: Intrinsic viscosity method

Density: BS 2782, Method 509A

tained by Test Method BS 2782, Method 105 C or ASTM D 123B. The molecular weight of the polypropylene is preferably below 100,000.

Preferably the molecular weight of the polyethylene is from 20,000 to 500,000 weight average, more preferably from 50,000 to 250,000.

The total weight of polymer in the grease is preferably 1-20%, more preferably 3-15% based on the total weight of the composition.

The weight ratio of atactic polypropylene to polyeth-

TABLE 2

| Oil | Kinematic Viscosity |       |       | Viscosity Index |
|-----|---------------------|-------|-------|-----------------|
|     | 100°F               | 140°F | 210°F |                 |
| Y   | 1077                | 242.6 | 41.33 | 76              |
| Z   | 137.2               | 40.49 | 10.27 | 43              |

TABLE 3

## DATA ON GREASES FROM ATACTIC POLYPROPYLENE B (MELT INDEX &gt; 50)

| Grease Ref. | Oil Type | Atactic Polypropylene |      | Polyethylene |       | Total Polymer % wt | Polypropylene :Polyethylene Ratio | Worked Pen. | Structure* | Notes                   |
|-------------|----------|-----------------------|------|--------------|-------|--------------------|-----------------------------------|-------------|------------|-------------------------|
|             |          | (B) % wt              | Type | Type         | % wt  |                    |                                   |             |            |                         |
| 4/1663      | Y        | 4.20                  | II   | 0.80         | 5.00  | 5.25 : 1           | 411                               | SI.G.SI.R   | )          | Grease can be smoothed, |
| 4/1663A     |          | 3.93                  | II   | 0.75         | 4.68  | 5.25 : 1           | 441                               | SI.G.SI.R   | )          | SI.R                    |
| 4/1661      | Y        | 4.20                  | III  | 0.80         | 5.00  | 5.25 : 1           | 442                               | SI.G        |            | Grease can be smoothed  |
| 4/1660      | Y        | 4.20                  | IV   | 0.80         | 5.00  | 5.25 : 1           | 436                               | SM          |            |                         |
| 4/1660A     |          | 3.93                  | IV   | 0.75         | 4.68  | 5.25 : 1           | 445                               | SM          |            |                         |
| 1/1739      | Z        | 9.98                  | II   | 1.98         | 11.96 | 5 : 1              | 401                               | G.SI.R      | )          | Grease can be smoothed, |
| 4/1668      |          | 7.43                  | II   | 1.48         | 8.91  | 5 : 1              | 410                               | G.SI.R      | )          | still                   |
| 4/1668A     |          | 5.81                  | II   | 1.16         | 6.97  | 5 : 1              | 473                               | G.SI.R      | )          | SI.R                    |
| 4/1669      | Z        | 8.75                  | III  | 1.75         | 10.50 | 5 : 1              | 372                               | G           | )          | Grease can be smoothed, |
| 4/1669A     |          | 7.66                  | III  | 1.53         | 9.19  | 5 : 1              | 411                               | G           | )          | with some               |
| 4/1669B     |          | 7.17                  | III  | 1.43         | 8.60  | 5 : 1              | 443                               | G           | )          | difficulty              |
| 1/1751      | Z        | 10.01                 | IV   | 1.98         | 11.99 | 5 : 1              | 420                               | SI.G        | )          | Grease can be smoothed, |
| 4/1667      |          | 8.75                  | IV   | 0.75         | 10.50 | 5 : 1              | 431                               | SI.G        | )          | easily                  |
| 1/1778      |          | 7.53                  | IV   | 3.67         | 11.00 | 2 : 1              | 401                               | SI.G        | )          |                         |
| 1/1769      |          | 6.67                  | IV   | 3.33         | 10.00 | 2 : 1              | 422                               | SI.G        | )          |                         |

\* NOTES:

SM = Smooth

G = Grainy

R = Rubbery

SI = Slightly

TABLE 4

## EFFECT OF MELT INDEX

| Grease Ref. | Oil Type | Atactic Polypropylene Type B |       | Worked Pen. | Structure* | Notes                      |
|-------------|----------|------------------------------|-------|-------------|------------|----------------------------|
|             |          | Melt Index Range             | % wt  |             |            |                            |
| 4/1629      | Y        | 0 - 20                       | 5.50  | 373         | G.R        | ) Very difficult to smooth |
| 4/1629A     |          | 0 - 20                       | 4.40  | 436         | G.R        | ) grease                   |
| 4/1630      |          | 20 - 50                      | 5.50  | 436         | SI.G.R     | Grease can be smoothed     |
| 4/1631      |          | >50                          | 5.50  | 443         | SI.R       |                            |
| 4/1657      |          | >50                          | 7.20  | 438         | SI.R       |                            |
| 4/1633      | Z        | 0 - 20                       | 15.00 | 173         | Vy.G.R     | ) Extremely difficult to   |
| 4/1633A     |          | 0 - 20                       | 9.40  | 364         | Vy.G.R     | ) smooth grease            |
| 4/1634      |          | 20 - 50                      | 15.00 | 398         | SI.G.R     | Grease can be smoothed     |
| 4/1634A     |          | 20 - 50                      | 11.30 | 440         | SI.G.R     | ) with some difficulty     |
| 4/1635      |          | >50                          | 15.00 | 420         | SI.R       | Grease can be smoothed     |
| 4/1454      |          | >50                          | 12.00 | 428         | SI.R       | )                          |

\* NOTES:

SI = Slightly

G = Grainy

Vy = Very

R = Rubbery

We claim:

1. A grease composition which consists essentially of a lubricating base oil thickened to a grease consistency with from 1 to 20% weight of a polymer mixture, said polymer mixture consisting of an atactic polypropylene of melt index above 50 and a molecular weight below 100,000, and a polyethylene of density above 0.94 grm./cc and molecular weight of 20,000 to 500,000, the weight ratio of said atactic polypropylene to polyethylene being from 1:1 to 10:1.

2. A grease composition as claimed in claim 1 in which the weight ratio of atactic polypropylene to polyethylene is from 2:1 to 5:1.

3. A grease composition as claimed in claim 1 in which the polyethylene has a molecular weight of 50,000 to 250,000.

4. A grease composition as claimed in claim 1 which has a penetration above 300.

5. A grease composition as claimed in claim 1 which has a penetration of 310 to 500.

\* \* \* \* \*

PO-1050  
(5/69)

UNITED STATES PATENT OFFICE  
CERTIFICATE OF CORRECTION

Patent No. 3,850,828

Dated December 11, 1974

Inventor(s) Stanley Charles Dodson & Robert Henry Newman

It is certified that error appears in the above-identified patent  
and that said Letters Patent are hereby corrected as shown below:

Column 2, line 15, please delete "mins."

Column 4, line 5, in Table 3 the subtitle "orked Pen." should  
read -- Worked Pen. --.

Signed and sealed this 28th day of January 1975.

(SEAL)  
Attest:

McCOY M. GIBSON JR.  
Attesting Officer

C. MARSHALL DANN  
Commissioner of Patents